

June 15, 1965

R. T. DAVIS, JR

3,188,734

METHOD OF MAKING CONTAINER STOCK

Filed Oct. 30, 1961



3,188,734

**METHOD OF MAKING CONTAINER STOCK**  
 Raymond T. Davis, Jr., Monroeville, Pa., assignor to  
 United States Steel Corporation, a corporation of New Jersey

Filed Oct. 30, 1961, Ser. No. 148,514  
 5 Claims. (Cl. 29—528)

This invention relates to the manufacture of black plate or tin plate for use in the fabrication of containers and, in particular, to a method for making plate which is protected against corrosion and discoloration, and carries a primer or final organic coating.

Black plate and tin plate as now made are used extensively in the fabrication of containers. To permit their prolonged storage by the purchaser prior to use, both require chemical treatment, black plate for corrosion resistance and tin plate for discoloration resistance. Prior to fabrication into cans, furthermore, they are both frequently lacquered on at least one side.

I have invented a novel method of making black plate and tin plate whereby the sheet-steel base, in the form of strip, is continuously coated with lacquer after initial cold-rolling to an intermediate gage and is then cold-rolled to final gage with the lacquer coating thereon. The result is a product protected against corrosion and discoloration and ready for fabrication into containers after lithographing if desired, without the necessity for cleaning, chemical treatment or oiling after final cold-reduction.

In the present preferred practice of my method, I cold-roll low-carbon steel strip to a thickness approximating that of conventional tin plate or black plate, about 0.010", and then, after electrolytically cleaning, annealing and temper-rolling it, I coat the strip electrolytically with tin if the product desired is tin plate. I then apply to the tin plate or to black plate without tinning, if that is the desired product, a coating of lacquer on one or both sides. The lacquer-coated strip is then passed through a lacquer-curing chamber wherein it is suitably heated and then coiled after cooling. I then cold-roll the lacquer-coated strip to a final thickness of about one half that of the strip after coating.

A complete understanding of the invention may be obtained from the following detailed description and explanation which refer to the accompanying drawing the single figure of which is a diagram illustrating the present preferred practice.

Referring now in detail to the drawing, low-carbon steel strip S is cold-rolled to a thickness of about 0.010" (corresponding to 90 pounds per base box) in a mill 10 of known type. The strip is next passed through a conventional electrolytic alkaline cleaning tank 11 and thence through a continuous annealing furnace 12, also of known construction. After cleaning and annealing, the strip is temper-rolled in a mill 13 where it is subjected to a reduction of only from 1 to 6%.

If the final product desired is tin plate, the strip is next passed through a continuous electrolytic tinning line 14, of known type. Thereafter, the strip is passed through a lacquer-coating line 15. If black plate is to be the final product, the tinning line is by-passed and the strip is sent from mill 13 directly to the lacquer-coating line.

In the line 15, the strip S is uncoiled and passed through a conventional roller coater 16 which applies a film of lacquer over the entire surface of one or both sides of the strip. The lacquer applied may be of any suitable type, examples of which are that made by Watson-Standard Company designated 17-926, a white cross-linked vinyl lacquer; and the oleo-resinous sanitary lacquer used by American Can Company. The lacquer is applied in thicknesses such as to afford a finished coating weight,

after curing but before further cold reduction, of from 4 to 11 mg./sq.in., conveniently about 7 mg./sq.in. After coating, the strip is passed through a heating chamber 17 where it is heated to a temperature from about 375 to 420° F. It is then cooled by contact with the atmosphere on emerging from chamber 17 and recoiled.

The lacquer-coated strip is next cold-rolled to effect about a 50% reduction in its thickness, i.e., from about 0.010" to about 0.005" (corresponding to 45 pounds per base box), by one or more passes through a reducing stand or stands 18, in accordance with usual cold-rolling practice. In this rolling, both the lacquer coatings and the base metal are reduced simultaneously in thickness but the coatings are not damaged nor is their adherence impaired. The finished product has a continuous uniform coating of lacquer strongly adherent thereto. The coating weight, of course, is reduced in proportion to the reduction in metal thickness but the rolling of the lacquer-coated strip presents no problem either of fragmentation of the coating or adherence thereof to the rolls. The product is well suited as such for fabrication into containers immediately or after further lacquering and lithographing if desired.

The advantages of my method are the economies in manufacture resulting therefrom. As stated, the conventional cleaning subsequent to final cold-rolling is made unnecessary, and the chemical treatment and oiling may be avoided in the production of tin plate. The chemical treatment is also eliminated from the operations which have been required in the manufacture of black plate. The lacquer coating, of course, protects black plate from corrosion and tin plate from discoloration and abrasion. The efficiency of the use of lacquer is increased, since the amount of lacquer which has been used heretofore covers twice as great an area of product, either tin plate or black plate.

Although I have disclosed herein the preferred practice of my invention, I intend to cover as well any change or modification therein which may be made without departing from the spirit and scope of the invention.

I claim:

1. A method of making container stock comprising cold-rolling low-carbon steel strip to a thickness greater than that desired in the finished product, applying a lacquer coating to the strip, thermally curing the lacquer coating, and cold-rolling the lacquer-coated strip thereby reducing its thickness to final gage.

2. A method as defined in claim 1, characterized by applying said coating in a thickness such as to result in a coating weight of from 4 to 10 mg. per square inch on one side only.

3. A method as defined in claim 1, characterized by applying said coating to both sides of said strip.

4. A method as defined in claim 1, characterized by reducing said strip by said first cold-rolling to a thickness of about 0.010" and by said second cold-rolling to a thickness of about 0.005".

5. A method of making lacquered steel strip comprising cold-rolling strip to intermediate gage, lacquering the strip, then cold-rolling it to final gage and effecting a substantial reduction in the strip thickness by said final cold-rolling.

#### References Cited by the Examiner

#### UNITED STATES PATENTS

- 1,898,739 2/33 Meyer ----- 29—527 X  
 2,850,999 9/58 Kaplan et al. ----- 29—528 X  
 3,110,413 11/63 McKay et al. ----- 29—528 X

70 WHITMORE A. WILTZ, Primary Examiner.

HYLAND BIZOT, Examiner.